

June 15, 1965

H. LASKE

3,188,735

METHOD FOR PRODUCING VERY THIN AND BRIGHT METAL WIRES AND PROFILES

Filed June 2, 1961

FIG.1



FIG.2



FIG.3

UNCOATED  
WIRE

COATED  
WIRE

DRAWING  
DIE #1

DRAWING  
DIE #2

PASSING ELECTRIC  
CURRENT THROUGH  
THE COATED WIRE  
TO EVAPORATE  
THE COATING

by

Jacob S. Kollin,  
ATTORNEY

HANS LASKE

3,188,735

**METHOD FOR PRODUCING VERY THIN AND BRIGHT METAL WIRES AND PROFILES**

Hans Laske, Luruper Chaussee 73, Hamburg-Bahrenfeld, Germany

Filed June 2, 1961, Ser. No. 114,555

 Claims priority, application Germany, June 27, 1960,  
 L 36,437

2 Claims. (Cl. 29—529)

The invention relates to an improved method and means for producing very thin stretched metal profiles such as thin wires, strips, bands, and the like, by drawing or rolling those profiles when coated with some material facilitating the drawing or rolling process, which material is removed after the reducing procedure. Heretofore, in the employment of the coating metal was removed by means of acids or alkalines.

The present application is a continuation-in-part of my copending U.S. application Serial No. 30,863, filed on May 23, 1960, now abandoned. In that application there was disclosed, by way of example, a method for producing very thin and bright metal wires, especially wires having a diameter of less than 0.00005 inches. The method and means for carrying it out are equally well applicable to all very thin stretched metal profiles, as above mentioned, and not only to wires.

Such wires could heretofore be produced, e.g. by means of the Wollaston method. In this method the wires to be drawn are first coated, e.g. by electro-plating with a metal coat. After the wires have passed one or more dies the coat which facilitates the drawing is removed by means of acids or alkalies, which makes bright wires.

One object of the invention is a new method for producing very thin and bright metal profiles, such as wires in which the latter are not at all contacted with any corrosive medium such as acid, lye, oxygen or other chemical substances and in which any subsequent neutralizing steps are obviated.

Another object of the invention is to produce bright metal wires having diameters less than attainable with the presently known methods.

According to the present invention the metal profile to be treated consisting e.g. of iron or nickel is coated with a metal or non-metallic material the vaporization temperature of which is below the melting point of the material to be processed. The profile is then reduced, e.g. by drawing or rolling in a manner known per se and afterwards the coating is removed by vaporization of the coating material to leave a bright surface.

It is well known in the practice of drawing or rolling, to use for the coating a metal e.g. zinc or cadmium. The present method includes the use of tin and lead as coating materials. In the present invention it is essential that the vaporization temperature of the coating material and the melting temperature of the material to be processed shall be sufficiently different so that the material to be processed will not be affected by the vaporization step.

In order to avoid high vaporization temperatures it is advisable to effect the vaporization in a vacuum chamber i.e. at lower temperatures.

Another object of the present invention is to provide the heat for the vaporization of the coating material by conducting an electric current through the material to be processed.

If fine wire resistors enveloped in closed bulbs have to be produced, the coated wires with connecting electrodes are mounted in the bulb before the vaporization step of the coating material, and then the coating material is vaporized by passing a heating current through the wire.

Furthermore, it is part of the present invention that the condensation of the vaporized coating material, espe-

cially if this is a metallic one, is limited to predetermined areas of the envelope or bulb by differently cooling and heating the latter. The heating may be done by HF-heating coils and the cooling by cooling jackets slipped over the envelope or bulb.

Further details and features of the present invention will become apparent from the following description and the attached drawing, which show preferred embodiments.

10 In the drawings:

FIGURE 1 is a cross-section through a vacuum chamber for vaporizing the coating material and

FIGURE 2 is a schematic view of an electric heating system for fine wires enveloped in a closed bulb.

FIG. 3 is a flow sheet of the claimed process.

As shown diagrammatically in the drawing the thin metal wire is conducted through an electro-plating bath in which the coating material having a vaporization point substantially lower than the melting point of the wire is deposited on the wire. The coated wire is drawn successively through a number of dies until it is reduced to the desired thickness. The wire is next connected across a pair of electrodes, in a container. An inert gas is introduced into the container and the latter is closed. Current is passed through the coated wire, sufficient to vaporize the deposited coating without melting the wire proper. The wire freed of the coating is then removed from the container.

As may be seen from the drawings, for the performance 30 of the present invention it is necessary to provide a vacuum chamber **a** with a suction pump **b**, said chamber comprising heating elements **c** for heating the coated wires **d**, coils or the like up to the vaporization point of the coating material. The coated and, e.g. already, coiled wire **d** is put into the vacuum chamber **1** for vaporizing the coating material.

According to the size of such vacuum heating chamber it is possible to handle larger or smaller quantities of such wires or even ready-made resistors.

FIGURE 2 shows a fine wire stretched out in a bulb of glass when vaporizing the coating material.

In this figure the resistor wire **11** already drawn and still coated with the material facilitating the drawing procedure is provided with thicker electrodes or mounting wires **12** and **13** at its both ends.

Preferably before the last drawing step the mounting wires **12** and **13**, respectively, are connected to the ends of the resistor wire.

By means of the mounting wires **12** and **13** the resistor wire **11** has been fused into the glass bulb and the projection **15** of the glass bulb **14** is closed by melting after the filling of the bulb **14** with some protective gas or the like.

To prevent oxidation during the vaporization procedure 55 it is possible to use a special inert gas which after vaporization of the coating may be removed and replaced by such gas as e.g. hydrogen which is required for the use of the resistor.

The vaporization of the material coating the wire **11** is performed by closing the switch **16** so as to direct a current from the source **17** through the wire **11**, the current being controlled by a resistor **18** in conjunction with the ammeter **19**.

To prevent an uncontrolled condensation of the vaporized coating material on the walls of the bulb **14** and, 65 when a metallic coating material is used, to avoid short-circuiting effects between the two wires **12** and **13** through the condensation deposits, the cross-section of the bulb portion surrounding the wires **12** and **13** is substantially reduced so that coils **20** and **21** may be slipped over the bulb end-portions and connected directly to an HF-current generator **22** for creating within the bulb **14** so high a

temperature that any condensation at such locations will not be possible.

In the case when the connecting or mounting wires for the resistor are provided at one end of the bulb only, only one inductor coil will be necessary for the prevention of the condensation. Further, in the shown embodiment, it is possible to omit one of the inductor coils if a capacitive influence on the resistor by a jacket of condensed coating metal is of no importance.

To direct the condensation of the vaporized coating material to certain parts of the wall of the bulb it is possible to provide at these parts an additional cooling, e.g. the cooling jacket 23 as shown in the drawings.

Instead of heating the wire 11 by the passage of a direct current it is also possible to induce a flow of current by means of a transformer or by causing an eddy current to flow in the conductor 12 by means of external HF-heating means.

The envelope or bulb of the resistor need not necessarily be of insulating material but may be of metal from which the connecting wires 12 and 13 are insulated.

Instead of a metallic coating material some insulating material with correspondingly low vaporization temperature may be used.

The method according to the invention is not restricted to wires but may be adopted for other thin stretched metal profiles, e.g. thin profiles such as strips and bands as transparent foils for capacitive surface illumination by electro luminescence may be produced by the described method. Further very thin metal strips or small metal plates to be used for electrostatic screening and as a contrast filter in the production of cathode ray tubes may also be produced.

What I claim is:

1. Apparatus for vaporizing a protective coating from very thin and bright metal wires comprising an airtight container which is provided with a pair of spaced electrodes adapted to be connected to the respective ends of a wire, for vaporizing a protective coating previously applied, a low frequency electric current supply connected to said electrodes, the portion of the container enclosing said electrodes being of a reduced cross-section, said apparatus comprising at least one high frequency coil for enclosing said portion, a high frequency generator connected to said coil, said generator being adapted to generate a high temperature in said end portion to thereby

4  
prevent condensation of the vaporized coating material on the walls of said container.

2. A method of producing very thin stretched metal profiles, such as thin wires, strips, bands and the like, to be employed as resistors, comprising coating the surface of a thin metal profile having a predetermined melting point with a metallic coating material having a predetermined vaporization point substantially lower than the melting point of the metal profile, so as to provide a coated thicker metal profile; reducing the cross-section of the coated profile by drawing the latter through a number of dies, connecting the respective ends of the profile to a pair of electrodes, fusing the electrodes to a container, introducing an inert gas into the container, closing the container, removing the coating material from the surface of the metal profile by passing electric current therethrough of a strength sufficient to heat the profile beyond the vaporization point of the coating material while cooling the container during the step of vaporization to thereby direct the condensation of the vaporized coating material to predetermined parts of the container wall and removing the inert gas after the vaporization of the coating.

References Cited by the Examiner

UNITED STATES PATENTS

|           |       |                   |             |
|-----------|-------|-------------------|-------------|
| 669,698   | 3/01  | Ivins.            |             |
| 930,723   | 8/09  | Von Bolton        | 29—198 X    |
| 1,026,383 | 5/12  | Coolidge          | 29—424 X    |
| 1,071,174 | 8/13  | Von Pirani et al. | 205—21      |
| 1,082,933 | 12/13 | Coolidge          | 29—420.5 X  |
| 1,273,506 | 7/18  | Lederer           | 205—21      |
| 1,345,441 | 7/20  | Hisamoto          | 205—21      |
| 1,597,189 | 8/26  | Gero              | 29—198 X    |
| 1,700,454 | 1/29  | Schumacher.       |             |
| 1,948,485 | 2/34  | Anselm            | 29—528 X    |
| 2,100,697 | 11/37 | Loewe             | 219—10.41 X |
| 2,447,979 | 8/48  | Hensel et al.     |             |
| 2,721,372 | 10/55 | Levi              | 29—424 X    |
| 2,866,262 | 12/58 | Mataich           | 29—424 X    |
| 2,913,561 | 11/59 | Rummel et al.     | 219—10.43   |
| 2,930,879 | 3/60  | Scatchard.        |             |

45 WHITMORE A. WILTZ, Primary Examiner.

HYLAND BIZOT, JOHN F. CAMPBELL, Examiners,